

# United States Patent Office

2,970,935

Patented Feb. 7, 1961

1

2,970,935

## METHOD OF RINSING METALLIC SURFACES WITH SOLUTIONS CONTAINING HEXAVALENT CHROMIUM

Walter A. Cavanagh, Detroit, Mich., assignor to Parker Rust Proof Company, Detroit, Mich., a corporation of Michigan

No Drawing. Filed Mar. 2, 1959, Ser. No. 796,218

7 Claims. (Cl. 148—6.16)

This invention relates to improvements in the method of operating hexavalent chromium containing rinse solutions on a continuous basis and more particularly relates to improvements in the method of formulating dilute hexavalent chromium containing solutions and continuously operating such solutions as rinses for improving the corrosion resistance of metallic surfaces and chemically coated metallic surfaces.

The utility of the hexavalent chromium ion in aiding the corrosion resistance of metal surfaces is well known and particularly in the art of chemically coating metals with a phosphate, oxalate, sulphide or similar coating, the use of a final dilute aqueous rinse containing hexavalent chromium ion is widely practiced. U.S. Patent 2,067,216 taught the use of solutions of this type for the purpose of improving the receptivity of a chemically coated metal surface for paint and specifically included the use of mixtures of chromic acid and phosphoric acid. Since this teaching, a large number of specific hexavalent chromium ion containing solutions have been used, each varying slightly from the other and compounded to achieve optimum improvement in corrosion resistance or paint base receptivity, for specific types of metallic surfaces or chemically coated metallic surfaces. Phosphate coatings, for example zinc phosphate and alkali metal phosphate coatings are soluble in certain hexavalent chromium containing solutions and in fact can be completely stripped from a metallic surface by a highly acidic hexavalent chromium containing solution. For this reason it has been customary to carefully control the acidity of the dilute aqueous hexavalent chromium containing rinse solution, and in continuous operation the maintenance of such a solution has been effected by periodically determining the free acid concentration of the rinse solution. As the rinse is used, sufficient water is added to maintain the rinse solutions bath level and chromic acid is added to preserve the free acid at approximately its original concentration. It has been found that in certain installations this procedure upon continued use results in the rinse causing staining of the surface, and in other installations the identical procedure ultimately results in the rinse losing its effectiveness in enhancing corrosion resistance or improving the receptivity of the surface for paint, lacquer or the like.

In accordance with this invention it has now been found that the above difficulties can be completely avoided, and the continuous operation of dilute aqueous hexavalent chromium containing rinse solutions rendered uniform in effectiveness by concurrently controlling the free acidity, the total acidity and the hexavalent chromium ion concentration of such solution, instead of merely controlling free acidity thereof. The basic discovery upon which the present invention rests is that the addition of water to the operating rinse solution has an important effect on the free acidity of the rinse solution depending upon the alkalinity of that water which is added. Heretofore it has been suggested that the use of hard water in rinse solutions of this type should be avoided but in accordance with this invention it has been found that a much more important characteristic of these replenishing waters is the alkalinity of the

2

water. The expression "alkalinity of the water" refers to the amount of acid solution which is required to neutralize the water to a pH close to that desired for use as a rinse solution. This alkalinity figure is conveniently expressed in parts per million of calcium carbonate and is determined for any particular water by titrating a 100 ml. sample of the water with N/50  $H_2SO_4$  using methyl orange as the indicator, which procedure titrates the water of a pH of approximately 4.3. The titration in ml. of  $H_2SO_4$  multiplied by 10 is the alkalinity in parts per million of calcium carbonate. This alkalinity figure can be used to formulate a desired hexavalent chromium ion containing rinse to contain any given desired concentration of  $CrO_3$  and having the desired free acidity and total acidity. The makeup of such solutions will be discussed more in detail hereinbelow.

The free acidity of the dilute aqueous hexavalent chromium ion containing rinse solutions of this invention should fall within the range of about 0.05 to about 1.0.

As used in this specification and in the appended claims, the expression "free acidity" refers to the number of ml. of N/10 sodium hydroxide which is required to titrate a 25 ml. sample of the rinse solution to a brom-cresol green end point. The number of ml. is the points of free acidity. The solutions of this invention preferably have a free acidity within the range of about 0.1—0.5 and the most consistent results are attained when the free acidity is maintained with the range 0.2—0.4.

As above indicated, the concentration of the hexavalent chromium ion must be controlled within a range which will provide adequate corrosion enhancement and will nevertheless cause no staining on the particular work being rinsed therein. Staining, as understood by those skilled in the art, results from the uneven concentration of the hexavalent chromium ion on a localized portion of a surface being rinsed and can be visibly detected as a slight yellow to yellow color. Such a stain is particularly undesirable for surfaces which are to be subsequently painted because the stain shows through the subsequent paint layers as a different shade of the resulting final painted surface. While the resistance to corrosion, which is obtained, is not due solely to the concentration of the hexavalent chromium ion in the solution, it is necessary for consistent results to insure that the concentration of the hexavalent chromium ion does not go below a minimum threshold value. It will also be apparent that as the minimum threshold value is approached the maintenance of the solution above the threshold, as hexavalent chromium ion is depleted from the rinse solution both as a result of interaction with the metal surface and dragout, is a difficult matter and requires constant attention. It is therefore desirable to operate at a concentration substantially above the minimum value. The rinse solution should have a hexavalent chromium ion concentration, expressed as percent of  $CrO_3$ , weight/volume, of at least about 0.01%, and the concentration preferably is maintained within the range of about 0.04%—0.05%. The upper concentration of  $CrO_3$  is, as above indicated, the concentration which is slightly below that which will cause staining for the particular work being processed therethrough and for conventional commercial applications a concentration as high as about 0.1% is permissible. Where the treated surface is not to be subsequently coated with paint or the like and staining is of less concern, the concentration of chromic acid may exceed the 0.1% concentration.

When the free acidity approaches or exceeds the upper limit of about 1.0, certain chemical coatings and particularly zinc phosphate coatings are susceptible to being stripped and in this event the rinse solution becomes contaminated with the zinc phosphate stripped coating materials. In addition to consistently maintaining the free acidity and chromic acid concentration within the

above given ranges, it is important in order to obtain consistent corrosion resistance enhancement to operate the solution within a total acid range of about 0.5-10.0 and preferably in the total acid range of 3-7. As used in this specification and in the appended claims, the expression "total acid" refers to the number of ml. of N/10 sodium hydroxide which is required to titrate a 25 ml. sample of the rinse solution to a phenolphthalein end point and the number of ml. so used is the total acid point value of the solution.

The hexavalent chromium ion concentration of the rinse solutions of this invention is preferably obtained by using chromic acid to formulate the solutions, but the hexavalent chromium ion can be obtained by employing any of the metallic dichromates, such as, for example, sodium, ammonium, calcium, zinc, aluminum, and cobalt dichromates, etc. The use of metallic dichromates or an admixture with  $\text{CrO}_3$  is preferred in the material used to replenish the rinse solutions in this invention, and is necessary in all cases in which the addition of only chromic acid to return the operating rinse solution to substantially its original free acidity will cause the hexavalent chromium ion concentration to decrease in the solution. In such case, a portion of the hexavalent chromium ion, at least, is added as a metallic dichromate. The alkali metal dichromates being relatively inexpensive and easily obtainable, are preferred for this purpose, but it will be appreciated that the use of other metallic ions may be more desirable in certain instances, depending upon the type of chemical coating which may be present on the surface that is being rinsed. For example, the provision of the hexavalent chromium ion as zinc dichromate is desirable when the chemical coating on the surface being rinsed is a zinc phosphate coating, etc.

The free acidity of the solution may be adjusted as needed, by adding to the solution either chromic acid or phosphoric acid and as above indicated when the hexavalent chromium ion concentration has decreased below that desired, the replenishment of the hexavalent chromium ion concentration by using chromic acid is preferred. However, when the restoration of the free acidity with chromic acids will cause the hexavalent chromium ion to exceed the desired level, the free acidity may be restored by adding phosphoric acid or a mixture of phosphoric acid and chromic acid and for this purpose a desirable admixture contains approximately equal parts of phosphoric acid and chromic acid.

It is also to be understood that in instances in which the replenishment of hexavalent chromium ion concentration of the solution with  $\text{CrO}_3$  raises the free acidity above the desired level, that the free acidity which is desired can be obtained by adding a metallic carbonate to the solution for example, sodium, ammonium, potassium or calcium carbonate and for this purpose calcium carbonate has been found to be particularly desirable.

In preparing a dilute aqueous hexavalent chromium ion containing rinse solution to a particular desired concentration of  $\text{CrO}_3$  and a specific free acidity and total acidity, the first step is to establish the alkalinity of the water to be employed. It is only necessary then to add sufficient phosphoric acid to the particular quantity of water employed in the particular solution to neutralize the alkalinity of the water to a pH of about 4.3 or, as above indicated, to the methyl orange end point. The desired hexavalent chromium ion concentration, expressed as  $\text{CrO}_3$ , is then obtained by adding sufficient dichromate or dichromate mixed with  $\text{CrO}_3$  to the neutralized solution to secure that desired concentration. The effect of the alkalinity of the water on the free acidity of the resulting solution is clearly illustrated in the following example. The addition of 0.1 gm./1 of  $\text{CrO}_3$  to distilled water produces a solution containing 0.01%  $\text{CrO}_3$  and having a free acid of 0.3 point. In order to obtain a solution having the same free acid when the water is one having an alkalinity of 300 p.p.m. it is necessary to add

0.6 gm./1 of  $\text{CrO}_3$  and this solution has a  $\text{CrO}_3$  content of 0.06%. It will be apparent, therefore, that in the operation of a rinse solution in a location in which the water added to maintain the rinse solution level is substantially free of alkalinity, as is distilled or deionized water, that maintenance of a  $\text{CrO}_3$  concentration in the preferred range of 0.2%-0.4%  $\text{CrO}_3$  by replenishing with  $\text{CrO}_3$  will soon cause the free acid value to rise and finally will cause the free acid to exceed the upper limit of 1.0 and use of this material will strip chemical coatings on the metal surfaces being rinsed. If this practice is continued the contaminating dissolved coating will additionally cause the total acid to exceed its upper limit of 10.0. Such rinse solutions are satisfactorily continuously maintained, however, and within the above given limits by adding  $\text{CrO}_3$  in the form of a metallic dichromate, or an admixture of  $\text{CrO}_3$  and a metallic dichromate which contains insufficient  $\text{CrO}_3$  to detrimentally raise the free acid content of the solution.

20 A rinse solution which is replenished with highly alkaline water is preferably maintained by the addition of phosphoric acid together with the replenishing hexavalent chromium ion containing material. The amount of phosphoric acid which is necessary is that quantity which is required to neutralize the alkalinity in the replenishing water to a pH of about 4.3, and for this purpose an ideal replenishing material is a mixture of phosphoric and chromic acids.

25 In the continuous operation of rinse solutions which are replenished with alkaline water the alkalinity of the water can be satisfactorily counteracted by employing quantities of 75% phosphoric acid, per liter of the alkaline water, in proportion to the alkalinity of that water with reference points as follows: for 100 p.p.m. alkalinity 30 water add 0.25 gm. of 75%  $\text{H}_3\text{PO}_4$ ; for 200 p.p.m. alkalinity water add 0.5 gm. of 75%  $\text{H}_3\text{PO}_4$ ; for 300 p.p.m. alkalinity water add 0.75 gm. of 75%  $\text{H}_3\text{PO}_4$  and for 400 p.p.m. alkalinity water add 1.0 gm. of 75%  $\text{H}_3\text{PO}_4$ . The addition of these quantities of phosphoric acid per liter of the water used to restore the rinse solution level has been found to completely counteract the effect of alkalinity on the maintenance of the rinse solution in uniform corrosion resistance enhancement condition as it is used to rinse either bare metal surfaces or chemically coated metal surfaces. In either type of rinsing operation, some of the chromic acid is used up in reaction with the metal surface or with the chemical coating on that surface and some of the  $\text{CrO}_3$  is lost by drag-out on the surface being coated. In practice it has 40 been found that sufficient  $\text{CrO}_3$  is removed in this manner that when the alkalinity of the water is counteracted completely by the phosphoric acid addition, as above explained, a highly satisfactory replenishing material for restoring the  $\text{CrO}_3$  concentration to its desired level, is 45 one containing 10-25%  $\text{CrO}_3$ , and 90-75% of a metallic dichromate, preferably calcium dichromate. The addition of a quantity of this hexavalent chromium ion containing admixture sufficient to restore the  $\text{CrO}_3$  level to its original concentration, additionally restores the free 50 acidity which was lost during rinsing by virtue of both drag-out and reaction with the surface, as above explained.

The rinse solutions of this invention can be applied by any of the conventional procedures including spraying, brushing or flowing the solution on the surface to be rinsed, or the article can be dipped in the solution at temperatures between room and slightly below boiling, preferably at about 120° F.-150° F. The replenishing materials are added at intervals sufficiently short so that the free acidity,  $\text{CrO}_3$  concentration, and total acidity remain at all times within the above given limits and preferably near to their initial values.

The following specific example illustrates, in greater detail, the original makeup and the replenishing of a

hexavalent chromium ion containing rinse solution in accordance with this invention, but it is to be understood that the specific concentrations of the ingredients and the conditions used therein are illustrative only and are not intended to be definitive of the operating limits of this invention.

The water to be used in the rinse solution was first analyzed and found to contain 150 parts/million of alkalinity. A 1,000 gallon solution was prepared by admixing 3.12 lbs. of 75%  $\text{H}_3\text{PO}_4$  and 4.57 lbs. of an admixture containing 75% calcium dichromate and 25%  $\text{CrO}_3$  by weight, with sufficient water to form 1,000 gallons. Upon analysis the solution was found to have a  $\text{CrO}_3$  content of 0.04%, a free acidity of 0.24 point and a total acidity of 2.0 points.

Steel sheets, in the form of automobile fenders, ultimately intended to be painted, were first coated with a zinc phosphate coating of conventional type and thereafter rinsed in the rinse solution by spraying at 120° F.-130° F. with conventional spray apparatus. At the end of 4 hours operation, the rinse solution had been replenished with 100 gallons of 150 p.p.m. alkalinity water and an analysis indicated that the solution then had a free acidity of 0.13 point, a total acidity of 1.9 points and a  $\text{CrO}_3$  concentration of 0.035%. The rinse solution was replenished by adding thereto 0.31 pound of 75%  $\text{H}_3\text{PO}_4$  and 5.6 pounds of the calcium dichromate- $\text{CrO}_3$  admixture used in the makeup of the rinse solution. An analysis of the rinse solution after replenishing, indicated that the free acidity had been restored to 0.24 point, the total acidity was 2.3 and the  $\text{CrO}_3$  concentration was restored to the original 0.04%. Continued operation of the rinse solution under similar conditions required subsequent replenishing with similar quantities of 75%  $\text{H}_3\text{PO}_4$  and the admixture of calcium dichromate and  $\text{CrO}_3$  for each 100 gallons of water added to maintain the level of the rinse solution. The addition of these quantities to the rinse solution maintained its free acidity and its  $\text{CrO}_3$  concentration at substantially the initial values and the quality of the receptivity for paint remained high and was completely satisfactory.

What is claimed is:

1. A method for maintaining an aqueous acidic hexavalent chromium containing solution in condition to enhance the corrosion resistance of metallic parts being continuously processed therethrough which comprises the steps of establishing an aqueous solution consisting essentially of about 0.01% to about 0.1%  $\text{CrO}_3$  and having a free acid in the range of about 0.05 to about 1.0 and a total acid in the range of 0.5-10.0 and as water is added thereto during use, maintaining the free acidity thereof within the above given range by adding thereto an acid selected from the group consisting of chromic acids and phosphoric acids, maintaining the  $\text{CrO}_3$  concentration within the above given range by adding thereto at least one hexavalent chromium ion-containing material and operating said rinse within the total acid concentration range of 0.5-10.

2. A method for maintaining an aqueous acidic hexavalent chromium containing solution in condition to enhance corrosion resistance of chemically coated metallic parts being continuously processed therethrough which comprises the steps of establishing an aqueous solution which consists essentially of about 0.01% to about 0.1%  $\text{CrO}_3$  and having a free acid in the range of about 0.05 to about 1.0 and a total acid in the range of 0.5-10.0, and as water is added thereto during use, maintaining the free acidity thereof within the above given range by adding thereto an acid selected from the group consisting of chromic acid and phosphoric acid, maintaining the  $\text{CrO}_3$  concentration within the above given range by adding thereto at least one hexavalent chromium ion-containing material and operating said rinse within the total acid concentration range of 0.5-10.

3. A method for maintaining an aqueous acidic hexavalent chromium containing solution in condition to enhance corrosion resistance of chemically coated metallic parts being continuously processed therethrough which comprises the steps of establishing an aqueous solution which consists essentially of about 0.01% to about 0.1%  $\text{CrO}_3$  and having a free acid in the range of about 0.05 to about 1.0 and a total acid in the range of 0.5-10.0, and as water is added thereto during use, maintaining the free acidity thereof within the above given range by adding thereto an acid selected from the group consisting of chromic acid and phosphoric acid, maintaining the  $\text{CrO}_3$  concentration within the above given range by adding thereto at least one hexavalent chromium ion-containing material selected from the group consisting of chromic acids and metallic dichromates and mixtures thereof, and operating said rinse within a total acid concentration range of 0.5-10.0.

4. A method for maintaining an aqueous acidic hexavalent chromium containing solution in condition to enhance corrosion resistance of metallic parts being continuously processed therethrough which comprises the steps of establishing an aqueous solution which consists essentially of about 0.04%-0.05%  $\text{CrO}_3$  and having a free acid in the range of 0.1-0.5 and, as water is added thereto, during use maintaining the free acidity thereof within the above given range by adding thereto an acid selected from the group consisting of chromic acid and phosphoric acid, maintaining the  $\text{CrO}_3$  concentration within the above given range by adding thereto a hexavalent chromium ion-containing compound, and operating said rinse within a total acid concentration range of 3-7.

5. A method in accordance with claim 3 wherein said hexavalent chromium ion-containing compound is an admixture of  $\text{CrO}_3$  and calcium dichromate containing 10-25%  $\text{CrO}_3$  and 75-90% calcium dichromate.

6. A method for maintaining an aqueous acidic hexavalent chromium containing rinse solution in condition to enhance the corrosion resistance of metallic parts being continually processed therethrough which comprises the steps of establishing an aqueous solution consisting essentially of about 0.01% to about 0.1%  $\text{CrO}_3$  and having a free acid in the range of about 0.05 to about 1.0 and as water is added thereto during use maintaining the free acidity thereof within the above given range by adding a quantity of phosphoric acid sufficient to neutralize the alkalinity of said water to a pH of 4.3, and maintaining the  $\text{CrO}_3$  concentration within the above given range by adding thereto a hexavalent chromium ion-containing compound selected from the group consisting of  $\text{CrO}_3$  and mixtures of  $\text{CrO}_3$  with at least one metallic dichromate, and operating said rinse within the total acid concentration range of 0.5-10.0.

7. A method in accordance with claim 6 wherein said alkalinity is neutralized by adding the equivalent of 75% phosphoric acid per liter of the said water added thereto with reference points as follows: 0.25 gram of 75%  $\text{H}_3\text{PO}_4$  for 100 p.p.m. alkalinity water; 0.5 gram of 75%  $\text{H}_3\text{PO}_4$  for 200 p.p.m. alkalinity water; 0.75 gram of 75%  $\text{H}_3\text{PO}_4$  for 300 p.p.m. alkalinity water; and 1.0 grams of 75%  $\text{H}_3\text{PO}_4$  for 400 p.p.m. alkalinity water.

#### References Cited in the file of this patent

#### UNITED STATES PATENTS

|           |                |               |
|-----------|----------------|---------------|
| 2,067,216 | Thompson       | Jan. 12, 1937 |
| 2,233,422 | Lodeeson       | Mar. 4, 1941  |
| 2,303,242 | Tanner         | Nov. 24, 1942 |
| 2,318,656 | Thompson       | May 11, 1943  |
| 2,391,656 | Tanner         | Dec. 25, 1945 |
| 2,403,426 | Douty et al.   | July 2, 1946  |
| 2,516,685 | Douty et al.   | July 25, 1950 |
| 2,609,308 | Gibson         | Sept. 2, 1952 |
| 2,882,189 | Russell et al. | Apr. 14, 1959 |